

## UNITED STATES PATENT OFFICE

2,523,917

AGE HARDENING AUSTENITIC  
ALLOY STEELS

Peter Payson, New York, N. Y., assignor to Crucible Steel Company of America, New York, N. Y., a corporation of New Jersey

No Drawing. Application November 2, 1949,  
Serial No. 125,173

8 Claims. (Cl. 75—124)

1

This invention pertains to age hardening austenitic alloy steels, and more particularly to an alloy steel of this type which can be forged, rolled or extruded, and which as annealed or solution-treated is relatively soft, so that it can be cold formed readily or machined, and which can be subsequently hardened to a hardness in excess of C35 and upward to C40 Rockwell for most analyses, and which possesses good corrosion resistance, and, as age hardened, high stretch resistance and high hardness both at room and elevated temperatures ranging up to 1350° F. or more. The steel of the invention is eminently suitable for use in automotive engine valves and valve parts, particularly the exhaust valves and valve parts thereof.

Although the heat hardening steel of my patent, Reissue 20,421, has been outstandingly successful for exhaust valves in automotive engines, it has the disadvantage of being relatively expensive owing to its high alloy content and high fabricating cost. Also, its resistance to stretching at elevated temperatures and its corrosion resistance in molten lead oxide are not as high as desired. In my Patent 2,484,903, I have described a further type of heat hardening steel suitable for automotive engine valves and valve parts, which is lower in alloy content, hence lower in cost, than the steel of my aforesaid patent, and which also is somewhat higher in corrosion resistance in molten lead oxide and higher in resistance to stretching at elevated temperatures than the steel of my patent, but, which, nevertheless, leaves something to be desired as to the latter characteristic.

Steels which are most resistant to stretching at the elevated temperatures to which automotive engine valves are subjected, ranging up to about 1350° F., are those possessing an austenitic structure. The heat hardenable steels are somewhat inferior by comparison in this respect because in the heat hardened state, they contain a considerable proportion of the sigma phase, which is a relatively hard and brittle constituent, and hence is less effective than austenite in imparting elevated temperature stretch resistance in steel. On the other hand, the austenitic steels are in general deficient in two vital respects as employed in automotive engine valves. They are not hard enough at relatively low temperatures for good wear resistance at the tappet end and

2

in the stem of the valve, and they are not hard enough at the elevated temperatures encountered in the automotive engine exhaust stream for wear resistance at the head, or seating surface, of the valve.

To overcome the first deficiency, it has been the practice to weld a stem of an ordinary hardenable steel, such as AISI 8640, to an austenitic steel head, and then to harden the stem end by 10 heat treatment. This involves a rather expensive resistance welding manufacturing operation. In some cases the stem and tappet end of a solid austenitic valve are hardened by cold working, but this again is an expensive manufacturing operation.

To overcome the second deficiency, it has been the practice to weld a deposit of a hard facing material, such as a high carbon, cobalt-chromium-tungsten alloy, to the seating surface of 20 the valve. This is so expensive an operation because of the high cost of both the hard facing material and the welding operation, that it is justifiable only for aeronautical, bus and truck engine valves.

25 The ideal material for exhaust valve service would be an austenitic steel of relatively low cost which could be hardened by heat treatment. The usual method of martensitic hardening of steel is not possible of course in an austenitic material. The only heat treatment method known for hardening such a steel is the precipitation hardening method, but although many precipitation hardening austenitic steels are known, very few are hardenable to the degree 30 required for valve steel service. It has been determined by many years of experience that for adequate service, the tappet end of an automotive engine exhaust valve should have a hardness of about Rockwell C38, or higher.

35 Some austenitic steels containing chromium, nickel, manganese and aluminum, which harden by precipitation to at least Rockwell C38 are described in my application, Serial No. 792,929, filed December 20, 1947; Serial No. 63,200 filed 40 December 2, 1948 and Serial No. 120,412 filed October 8, 1949, but all of these contain nickel over about 19%, and it is desirable from the 45 economic viewpoint that nickel be held to a minimum in a steel for automotive exhaust valves.

Now I have discovered that by employing and properly balancing the elements chromium, nickel, manganese and aluminum together with the carbon in steel, I can produce an austenitic steel that can be hardened by precipitation to at least Rockwell C38, while holding the nickel content thereof to a maximum of about 16%. Furthermore, this steel has the other desired properties for automotive exhaust valve service, namely, high resistance to corrosion in molten 10 lead oxide at temperatures up to 1675° F.; high resistance to stretching at temperatures up to

not have the wholly austenitic structure desired. On the other hand, since the hardness does not increase with increasing nickel above 14%, it is desirable from the economy viewpoint to hold the nickel to a maximum of about 16%.

The effect of chromium on the hardening of the steel may be seen from the test results in Table II.

Table II.—Effect of chromium on hardening

All samples solution treated at 2300° F. and aged 16 hours at the temperatures shown.

| Bar  | Analysis, Per Cent |     |     |      |      |     | Bal. | Rockwell "C" Hardness On Aging At— |          |          |
|------|--------------------|-----|-----|------|------|-----|------|------------------------------------|----------|----------|
|      | C                  | Mn  | Si  | Ni   | Cr   | Al  |      | 1200° F.                           | 1300° F. | 1400° F. |
| 2037 | .44                | 4.5 | .53 | 14.7 | 8.6  | 3.2 | Fe—  | 12                                 | 16       | 21       |
| 2251 | .48                | 4.7 | .63 | 14.7 | 10.3 | 3.3 | Fe—  | 21                                 | 37       | 34       |
| 2254 | .50                | 4.8 | .66 | 14.6 | 11.5 | 3.3 | Fe—  | 25                                 | 38       | 36       |
| 2257 | .52                | 4.8 | .70 | 14.6 | 13.6 | 3.3 | Fe—  | 35                                 | 39       | 37       |
| 2121 | .52                | 4.8 | .68 | 14.2 | 14.9 | 3.4 | Fe—  | 33                                 | 42       | 38       |

1350° F., under a stress of 1000 p. s. i.; and high hardness at exhaust valve service temperatures, as will be shown subsequently.

The steel of this invention has the following ranges of composition for "broad" and "preferred" analyses respectively:

|           | Broad Range           | Preferred Range       |
|-----------|-----------------------|-----------------------|
| Carbon    | about 0.40 to 0.80%   | about .50 to .60%     |
| Manganese | about 3.50 to 10.00%  | about 4.50 to 6.00%   |
| Silicon   | about 0.20 to 2.50%   | about .50 to 1.50%    |
| Nickel    | about 13.50 to 16.00% | about 14.00 to 15.00% |
| Chromium  | about 10.00 to 15.00% | about 12.00 to 14.00% |
| Aluminum  | about 2.50 to 4.00%   | about 3.00 to 3.50%   |
| Balance   | Substantially Iron    | Substantially Iron    |

In addition to the elements above specified, the steel of the invention may optionally also contain small amounts, i. e., up to about 5 or 6% in aggregate of other elements which enhance or at least do not impair the aforesaid properties of

These data show a marked increase in hardening of the 10.3% Cr steel compared with the 8.6% Cr steel, but only a very gradual increase in hardening in the steels ranging from 10.3% to 14.9% chromium. Therefore, the chromium in the steel of this invention should be at least about 10% but there is not much advantage in raising the chromium beyond about 15%, and from the viewpoint of economy about 12 to 14% is sufficient.

A minimum of about 2.5% manganese is required in the steel of the invention to assure that after it is aged it will be austenitic, that is, substantially non-magnetic. The hardening of the steel is not much affected by increasing the manganese beyond about 3.5% as shown by the test results in Table III.

Table III.—Effect of manganese on hardening

All samples solution treated at 2300° F. and aged 16 hours at the temperatures shown.

| Bar  | Analysis, Per Cent |     |     |      |      |     | Bal. | Rockwell "C" Hardness On Aging At— |          |          |
|------|--------------------|-----|-----|------|------|-----|------|------------------------------------|----------|----------|
|      | C                  | Mn  | Si  | Ni   | Cr   | Al  |      | 1200° F.                           | 1300° F. | 1400° F. |
| 2349 | .50                | 3.5 | .87 | 14.9 | 12.8 | 2.9 | Fe—  | 32                                 | 39       | 32       |
| 2350 | .53                | 4.8 | .90 | 14.7 | 12.7 | 3.0 | Fe—  | 36                                 | 41       | 35       |
| 2351 | .53                | 6.2 | .86 | 15.3 | 12.5 | 3.0 | Fe—  | 39                                 | 41       | 36       |
| 2352 | .54                | 7.8 | .42 | 14.9 | 12.4 | 3.0 | Fe—  | 39                                 | 43       | 35       |
| 2353 | .53                | 9.6 | .50 | 14.8 | 12.8 | 3.1 | Fe—  | 41                                 | 42       | 36       |

the steel. Thus nitrogen may be included up to about 0.3%, and any or all of such elements as vanadium, tungsten, molybdenum, cobalt and copper up to about 5% in aggregate.

When the nickel is under about 13% the steel does not harden adequately as may be seen from the test results in Table I below:

Table I.—Effect of nickel on hardening

All samples solution treated at 2300° F. and aged 16 hours at the temperatures shown.

Since manganese is not an expensive element I may use up to about 10% in the steel of the invention. However, the forceability of the steel becomes more difficult as the manganese is increased and I therefore prefer to keep the manganese at a maximum of about 6%.

Aluminum has a very important effect on the hardening of the steel because it is probable that the age hardening is caused by the precipitation of an aluminum compound. But the steel must contain an appreciable amount of aluminum, that

| Bar  | Analysis, Per Cent |     |     |      |      |     | Bal. | Rockwell "C" Hardness On Aging At— |          |          |
|------|--------------------|-----|-----|------|------|-----|------|------------------------------------|----------|----------|
|      | C                  | Mn  | Si  | Ni   | Cr   | Al  |      | 1200° F.                           | 1300° F. | 1400° F. |
| 2068 | .47                | 4.7 | .61 | 9.7  | 13.2 | 3.1 | Fe—  | 20                                 | 23       | 24       |
| 2071 | .47                | 4.7 | .62 | 12.1 | 13.2 | 3.2 | Fe—  | 19                                 | 28       | 32       |
| 5981 | .51                | 5.3 | .75 | 13.9 | 13.9 | 3.1 | Fe—  | 38                                 | 41       | 38       |
| 2257 | .52                | 4.8 | .70 | 14.6 | 13.6 | 3.3 | Fe—  | 35                                 | 39       | 37       |

Furthermore, the steels with less than about 13% Ni are somewhat magnetic after the high temperature solution treatment and therefore do

is, over about 2.5%, in order for the steel to develop adequate hardness for exhaust valve service, as may be seen from the test results in Table IV.

Table IV.—Effect of aluminum on hardening

All samples solution treated at 2300° F. and aged for 16 hours at the temperatures shown.

| Bar  | Analysis, Per Cent |     |     |      |      |     | Bal.    | Rockwell "C" Hardness On Aging At— |          |          |
|------|--------------------|-----|-----|------|------|-----|---------|------------------------------------|----------|----------|
|      | C                  | Mn  | Si  | Ni   | Cr   | Al  |         | 1200° F.                           | 1300° F. | 1400° F. |
| 2354 | .52                | 4.8 | .43 | 15.0 | 12.5 | 1.3 | Fe..... | 22                                 | 30       | 25       |
| 2355 | .52                | 4.7 | .43 | 15.0 | 12.4 | 2.2 | Fe..... | 27                                 | 32       | 23       |
| 2357 | .51                | 4.6 | .61 | 15.1 | 12.7 | 3.0 | Fe..... | 37                                 | 40       | 34       |

Since aluminum has a detrimental effect on the forgeability of the steel, I limit the aluminum content to a maximum of about 4%.

Silicon has a minor but definite effect on the hardening, as shown by the test results in Table V, and the steel should, therefore, contain a minimum of about 0.20% silicon. For satisfactory

this changed the hardness of several 0.15% C austenitic steels from Rockwell B90 to only B95 (Rockwell C9 to C16). It was therefore quite unexpected to find that carbon had the marked

effect on the hardness of the precipitation hardening steels of this invention as shown by the test results in Table VI below.

Table VI.—Effect of carbon on hardening

All samples solution treated at 2300° F. and aged for 16 hours, at the temperatures shown.

| Bar  | Analysis, Per Cent |     |     |      |      |     | Bal.    | Rockwell "C" Hardness On Aging At— |          |          |
|------|--------------------|-----|-----|------|------|-----|---------|------------------------------------|----------|----------|
|      | C                  | Mn  | Si  | Ni   | Cr   | Al  |         | 1200° F.                           | 1300° F. | 1400° F. |
| 2250 | .35                | 4.5 | .62 | 14.6 | 10.0 | 3.4 | Fe..... | 18                                 | 22       | 23       |
| 2251 | .48                | 4.7 | .63 | 14.7 | 10.3 | 3.3 | Fe..... | 21                                 | 37       | 34       |
| 2252 | .63                | 4.8 | .64 | 14.7 | 9.7  | 3.5 | Fe..... | 33                                 | 40       | 39       |
| 2253 | .33                | 4.8 | .67 | 14.6 | 11.8 | 3.3 | Fe..... | 21                                 | 31       | 25       |
| 2254 | .50                | 4.8 | .66 | 14.6 | 11.5 | 3.3 | Fe..... | 26                                 | 38       | 36       |
| 2255 | .62                | 4.7 | .68 | 14.7 | 11.6 | 3.4 | Fe..... | 35                                 | 39       | 39       |
| 2256 | .35                | 4.8 | .65 | 14.7 | 13.7 | 3.3 | Fe..... | 23                                 | 34       | 30       |
| 2257 | .52                | 4.8 | .70 | 14.6 | 13.6 | 3.3 | Fe..... | 35                                 | 39       | 37       |
| 2258 | .67                | 4.8 | .70 | 14.7 | 13.4 | 3.3 | Fe..... | 33                                 | 42       | 39       |
| 2119 | .33                | 4.8 | .63 | 14.0 | 14.6 | 3.4 | Fe..... | 23                                 | 36       | 31       |
| 2120 | .37                | 4.8 | .59 | 14.0 | 14.5 | 3.2 | Fe..... | 29                                 | 37       | 31       |
| 2122 | .47                | 4.8 | .68 | 14.2 | 14.9 | 3.4 | Fe..... | 33                                 | 42       | 38       |

forgeability, I limit the silicon in this steel to a maximum of about 2.5%, and preferably to 1.5%.

Table V.—Effect of silicon on hardening

All samples solution treated at 2300° F. and aged for 16 hours at the temperature shown.

It is evident from these data that the steel of this invention should have a minimum of about 0.40% carbon in order to harden to about Rockwell C38 after solution and aging treatments, and preferably a carbon content over 0.50%. However, in order to avoid difficulties in forging I

| Bar  | Analysis, Per Cent |     |     |      |      |     | Bal.    | Rockwell "C" Hardness On Aging At— |          |          |
|------|--------------------|-----|-----|------|------|-----|---------|------------------------------------|----------|----------|
|      | C                  | Mn  | Si  | Ni   | Cr   | Al  |         | 1200° F.                           | 1300° F. | 1400° F. |
| 2356 | .52                | 4.7 | .28 | 15.2 | 12.6 | 2.8 | Fe..... | 32                                 | 38       | 30       |
| 2357 | .51                | 4.6 | .61 | 15.1 | 12.7 | 3.0 | Fe..... | 37                                 | 40       | 34       |
| 2350 | .53                | 4.8 | .90 | 14.7 | 12.7 | 3.0 | Fe..... | 36                                 | 41       | 35       |

Finally, I have discovered that the carbon content of the steel of this invention is a very important factor in its hardening. Ordinarily, carbon is not considered of importance in precipitation hardening steels. It is, of course, known that carbon combines with many elements in steel to form carbides which have different degrees of solubility in austenite and which therefore can be dissolved and precipitated more or less at will by controlling the heating and the cooling of the steel. However, the precipitation of carbides in austenitic steel has very little effect on the hardness of the steel. For example, as stated in my paper, "Changes in Austenitic Chromium-Nickel Steels During Exposures at 1100 to 1700° F.," published in Trans. A. S. M. vol. 39, 1947, a heating for 200 to 900 hours at 1400° F. following a solution treatment at 2100° F. caused appreciable carbide precipitation but

40 limit carbon to a maximum of about 0.80%. Furthermore, with increase in carbon content, more and more chromium is combined permanently with carbon and it is necessary to increase the chromium in the steel to compensate for the higher carbon, and to retain the non-magnetic austenitic structure in the steel.

45 Although for purposes of uniformity the hardness data in all the tables above were determined with a solution treatment of 2300° F., I have established that the steel of this invention need not be solution treated at 2300° F. in order to be hardened. For example, the steel may be hardened from the as forged condition, or after a solution treatment at 2200° F., but the hardening after a 50 2100° F. treatment is not quite satisfactory as shown in Table VII.

Table VII.—Effect of solution treatment on hardening

Samples as forged and solution treated as indicated were aged for 16 hours at 1300° F.

| Bar  | Analysis, Per Cent |     |     |      |      |     | Bal.    | As Forged | Solution Treated At— |          |          |
|------|--------------------|-----|-----|------|------|-----|---------|-----------|----------------------|----------|----------|
|      | C                  | Mn  | Si  | Ni   | Cr   | Al  |         |           | 2100° F.             | 2200° F. | 2300° F. |
| 5979 | .51                | 3.9 | .73 | 14.0 | 14.0 | 3.1 | Fe----- | 39        | 35                   | 39       | 41       |
| 5981 | .51                | 5.3 | .75 | 13.9 | 13.9 | 3.1 | Fe----- | 41        | 33                   | 40       | 41       |

Evidently the hardening of the steel may depend on some cold working combined with some solution of precipitating compounds (the as forged condition) or on a high degree of solution of the compound (the 2200° F. and 2300° F. solution treatments). The treatment at 2100° F. apparently relieves the cold worked condition and does not effect sufficient saturation to cause adequate hardening during the subsequent aging.

As may be seen from the tables above, the optimum aging temperature for the steel of this invention is about 1300° F. but in many instances adequate hardness for valve service is also obtained by an aging treatment of 1400° F.

In spite of the low chromium content in the steel of this invention this steel has satisfactory resistance to corrosion in molten lead oxide as may be seen in Table VIII.

Table VIII.—Corrosion resistance in lead oxide at 1675° F.

| Bar  | Analysis, Per Cent |     |     |      |      |       |       | Bal.    | Loss, gms./sq. in. in 1 hr. |
|------|--------------------|-----|-----|------|------|-------|-------|---------|-----------------------------|
|      | C                  | Mn  | Si  | Ni   | Cr   | Al    | Mo    |         |                             |
| 2254 | .50                | 4.8 | .66 | 14.6 | 11.5 | 3.3   | ----- | Fe----- | 3.9-4.2-5.3                 |
| 2255 | .62                | 4.7 | .68 | 14.7 | 11.6 | 3.4   | ----- | Fe----- | 4.5-5.0-5.5                 |
| 2258 | .67                | 4.8 | .70 | 14.7 | 13.4 | 3.3   | ----- | Fe----- | 5.1-5.2-5.4                 |
| 5829 | .41                | 0.7 | .68 | 4.8  | 23.9 | ----- | 2.7   | Fe----- | 4.7-5.2-5.7                 |
| 2011 | .80                | 0.5 | 2.1 | 1.3  | 20.1 | ----- | ----- | Fe----- | 6.4-6.7-7.2                 |

Of the steels in Table VIII, the first three represent this invention; the fourth is a commercial valve steel of the sigma phase type, per Payson U. S. Patent Re. 20,421; and the fifth is a commercial valve steel of the martensitic type.

The stretch resistance of the steel of this invention is far superior to that of the two commercial valve steels mentioned above. As solution treated and aged to a hardness of Rockwell C38 to 40, the steel of this invention tested at 1350° F. with a stress of 10,000 p. s. i. elongated about 0.2 to 0.5% in 8 hours. Under these same testing conditions, the sigma phase valve steel represented by Bar 5829 of Table VIII elongated about 1.5% in 8 hours; while the martensitic valve steel represented by Bar 2011 of Table VIII stretched exceedingly and eventually ruptured in much less than 8 hours.

Finally, the steel of this invention as solution treated and aged to a hardness of Rockwell C38 to 40 has excellent hot hardness, having values of 215 to 255 Brinell at 1200° to 1400° F., in comparison with 175 to 200 Brinell for the sigma phase valve steel of Table VII; 120 to 150 for the martensitic type valve steel of Table VIII; and 105 to 140 for the austenitic 21% chromium-12% nickel type valve steel.

Thus on the basis of corrosion resistance, stretch resistance, hardness at elevated temperatures, as well as hardness at room temperature, the steel of this invention is eminently suitable for automotive engine exhaust valve service.

I claim:

1. A forgeable and machinable, age-hardenable, austenitic alloy steel which, on solution-treating at about 2300° F., followed by aging at

about 1300° F., is characterized in having a hardness in excess of "C" 35 Rockwell, said steel containing: about 0.4 to 0.8% carbon; about 13.5 to 16% nickel; about 3.5 to 10% manganese; about 10 to 15% chromium; about 0.2 to 2.5% silicon; about 2.5 to 4% aluminum; up to about 0.3% nitrogen; up to about 5% in aggregate of other elements which do not impair the age-hardening properties of the steel; and the balance substantially all iron.

2. A forgeable and machinable, age-hardenable, austenitic alloy steel which, on solution-treating at about 2300° F., followed by aging at about 1300° F., is characterized in having a hardness in excess of "C" 35 Rockwell, said steel containing: about 0.5 to 0.6% carbon; about 14 to 15% nickel; about 4.5 to 6% manganese; about 12 to 14% chromium; about 0.5 to 1.5% silicon; about 0.3% nitrogen; up to about 5% in aggregate of other elements which do not impair the age-hardening properties of the steel; and the balance substantially all iron.

3 to 3.5% aluminum; up to about 0.3% nitrogen; up to about 5% in aggregate of other elements which do not impair the age-hardening properties of the steel; and the balance substantially all iron.

3. An age-hardened austenitic alloy steel having a hardness in excess of "C" 35 Rockwell, said steel containing: about 0.4 to 0.8% carbon; about 13.5 to 16% nickel; about 3.5 to 10% manganese; about 10 to 15% chromium; about 0.2 to 2.5% silicon; about 2.5 to 4% aluminum; up to about 0.3% nitrogen; up to about 5% in aggregate of other elements which do not impair the age-hardening properties of the steel; and the balance substantially all iron.

4. An age-hardened austenitic alloy steel having a hardness in excess of "C" 35 Rockwell, said steel containing: about 0.5 to 0.6% carbon; about 14 to 15% nickel; about 4.5 to 6% manganese; about 12 to 14% chromium; about 0.5 to 1.5% silicon; about 3 to 3.5% aluminum; up to about 0.3% nitrogen; up to about 5% in aggregate of other elements which do not impair the age-hardening properties of the steel; and the balance substantially all iron.

5. A forgeable and machinable, age-hardenable, austenitic alloy steel which, on solution-treating at about 2300° F., followed by aging at about 1300° F., is characterized in having a hardness in excess of "C" 35 Rockwell, said steel containing: about 0.4 to 0.8% carbon; about 13.5 to 16% nickel; and about 3.5 to 10% manganese;

about 10 to 15% chromium; about 0.2 to 2.5% silicon; about 2.5 to 4% aluminum; and the balance iron.

6. A forgeable and machinable, age-hardenable, austenitic alloy steel which, on solution-treating at about 2300° F., followed by aging at about 1300° F., is characterized in having a hardness in excess of "C" 35 Rockwell, said steel containing: about 0.5 to 0.6% carbon; about 14 to 15% nickel; about 4.5 to 6% manganese; about 12 to 14% chromium; about 0.5 to 1.5% silicon; about 3 to 3.5% aluminum; and the balance iron.

7. An age-hardenable austenitic alloy steel having a hardness in excess of "C" 35 Rockwell, said steel containing about 0.4 to 0.8% carbon; about 13.5 to 16% nickel; about 3.5 to 10% manganese; about 10 to 15% chromium; about 0.2 to 2.5% silicon; about 2.5 to 4% aluminum; and the balance iron.

8. An age-hardenable alloy steel having a hardness in excess of "C" 35 Rockwell, said steel containing: about 0.5 to 0.6% carbon; about 14 to 15% nickel; about 4.5 to 6% manganese; about 12 to 14% chromium; about 0.5 to 1.5% silicon; about 3 to 3.5% aluminum; and the balance iron.

PETER PAYSON.

#### REFERENCES CITED

- 10 The following references are of record in the file of this patent:

#### UNITED STATES PATENTS

| Number    | Name           | Date          |
|-----------|----------------|---------------|
| 1,933,900 | Frevert et al. | Nov. 7, 1933  |
| 1,941,648 | Armstrong      | Jan. 2, 1934  |
| 2,127,245 | Breeler        | Aug. 16, 1938 |